

# UNITED STATES PATENT OFFICE.

HOWARD ANGELO MUTHS, OF MOBILE, ALABAMA.

## LEATHER-PRESERVER.

1,398,600.

Specification of Letters Patent. Patented Nov. 29, 1921.

No Drawing.

Application filed May 25, 1920. Serial No. 384,167.

To all whom it may concern:  
Be it known that I, HOWARD ANGELO MUTHS, a citizen of the United States, residing at Mobile, in the county of Mobile, State 5 of Alabama, have invented a new and useful Leather-Preserver; and I do hereby declare the following to be a full, clear, and exact description of the invention, such as will enable others skilled in the art to which it applies to make and use the same.

The invention relates to leather preservatives and has for its object to provide a preservative particularly adapted as a belt dressing to prevent belts from cracking or 15 burning, also to preserve the life of the belt and at the same time soften the belt and render the same flexible.

It has been found that a great number of the belt dressings now in use will cake or 20 gum upon the belts or pulleys and another objection to belt dressings is that they will pick up lint or waste material, which lint or waste material will cake on the belt and pulleys, therefore it is a further object of the 25 invention to provide a belt dressing to which waste materials will not adhere and at the same time a belt dressing which will not cake on the belt or pulleys.

With the above and other objects in view 30 the invention resides in the combination and arrangement of ingredients as hereinafter set forth, described and claimed, it being understood that changes in the precise embodiment of the invention may be made within 35 the scope of what is claimed without departing from the spirit of the invention.

I have found that by using the following 40 composition that the above results and objects may be obtained and that by using the following ingredients in the parts set forth that the best results are obtained. The ingredients and their quantities are as follows:

3 parts castor oil,

1 part paraffin or turpentine soap, 45  
1/4 part of Venetian turpentine or balsam fir,

1/4 part oil of cinnamon.

The above ingredients are placed in a receptacle and subjected to a cooking process 50 which is substantially as follows:—The paraffin or soap is heated and brought to a boil, then the castor oil is added and stirred thoroughly. The Venetian turpentine is then added at boiling point and finally the 55 oil of cinnamon. The composition is then taken from the fire and allowed to cool for 48 hours.

It has been found that a belt dressing comprising the above ingredients will not cake 60 on the belting or pulley and it has also been found that the belt will be thoroughly preserved and rendered flexible and prevented from cracking incident to drying out of the belt. It has also been found that waste and 65 foreign matter will not stick to a belt which has been treated to the above composition.

The invention having been set forth what is claimed as new and useful is:—

1. A composition of the character described comprising a mixture of castor oil, paraffin, Venetian turpentine, and oil of cinnamon.

2. A composition of the character described comprising a mixture three parts 75 castor oil, one part paraffin, one quarter part of Venetian turpentine and one sixty-fourth part of oil of cinnamon.

In testimony whereof I have signed my name to this specification in the presence of 80 two subscribing witnesses.

HOWARD ANGELO MUTHS.

Witnesses:

A. C. McCauley,  
Harry Havaller.